

Nov. 3, 1925.

1,559,572

C. KAPNER

METHOD OF PRODUCING ENAMELED METAL SIGNS

Filed June 12, 1925



INVENTOR  
*Charles Kapner*  
BY *N. J. Deulac*  
ATTORNEY

Patented Nov. 3, 1925.

1,559,572

# UNITED STATES PATENT OFFICE.

CHARLES KAPNER, OF BELLAIRE, OHIO.

## METHOD OF PRODUCING ENAMELED METAL SIGNS.

Application filed June 12, 1925. Serial No. 36,677.

To all whom it may concern:

Be it known that I, CHARLES KAPNER, a citizen of the United States of America, and resident of Bellaire, county of Belmont, and State of Ohio, have invented certain new and useful Improvements in Methods of Producing Enameled Metal Signs, of which the following is a specification.

This invention relates to a method of producing enameled metal signs, and it has for its primary object to provide a simple and comparatively inexpensive method of producing enameled-letter sheet-metal signs.

A further object is to provide a method of the character mentioned whereby an enameled metal sign embodying letters or characters to be prominently or conspicuously displayed may be produced with a minimum number of enamel coating and burning operations and, consequently, in a minimum of time and at a small fractional part of the expense heretofore involved.

In describing the invention in detail, reference is herein had to the accompanying drawing, in which—

The single figure is an elevation or plan view of a sign produced in conformity with my invention.

The sign is formed of sheet metal in a single, or unitary, structure, and consists of a pair of parallel bars 1 and 2, preferably of relatively narrow width, and sign letters or characters 3 formed between said bars. Said characters are made of skeleton form, the metal between adjacent letters being cut away to form open spaces 4, and the metal enclosed by, or located between, members of such letters being removed, as shown at 5.

For the purpose of rendering the letters or characters distinctly conspicuous, or so displayed that they may be readily discerned, the bars 1 and 2 are made of one color, as black, while the skeleton characters are made of a strongly contrasting color, as white. This coloring of the sign is effected by or through the application to the metal of colored coatings of enamel which, because of its glossy or lustrous light-reflecting character, is admirably adapted both for day and night display, and, further, because the enamel coating serves as a well-nigh perfect protection against deterioration of the metal.

In effecting the coating of the sign, a first, or base, coat of enamel of any desired color is applied to the sign surfaces, front

and rear, as by spraying or by dipping in a liquid enamel bath. This coating is then fired, or baked on, as ordinarily, following which a second coat of enamel is applied. 60 In case two coats are employed, the color of the second coat differs from that of the first coat, and the portion of the second coat applied to the bars 1 and 2 is removed, or wiped off, as by the use of a cloth or sponge, 65 so that the skeleton characters alone carry this second coat. The sign is then fired a second time for baking on the second coating.

A third coating of enamel may be, and 70 preferably is, applied to the sign, in which case the second coat is applied in the color which is to be borne by the bars 1 and 2 and no part thereof is removed. Then, immediately following the application of the 75 third coating, which shall be in a color contrasting with that of the second coat, the portion of the third coat borne by said bars is removed, following which the sign is fired to effect the burning or baking of the 80 third coating carried by the skeleton characters.

It will be understood that additional coatings of enamel may be separately applied and baked on, if desired; however, 85 satisfactory results are obtainable with three coatings, and but slightly less satisfactory results may be obtained with two coatings.

### What is claimed is—

1. The method of producing enameled metal signs, which consists in shaping a single sheet metal blank to form a pair of parallel bars and sign characters of skeleton form between and united at their ends to said bars, and then successively applying to 90 said bars and characters a base coating of enamel, baking said coating, applying a second coating of enamel in the color to be borne by said bars, firing this second coating, applying a third coating of enamel in 95 a contrasting color to be borne by said characters, wiping said third coating from said bars only, and finally baking the portion of said third coating borne by said characters.

2. The method of producing enameled metal signs, which consists in shaping a single sheet metal blank to form a unitary flat plate structure having portions cut therefrom to provide a pair of parallel horizontally disposed bars and a plurality of sign characters 105 of skeleton form located between and united at their tops and bottoms to said bars, and

then successively applying to the face of said plate a coating of enamel, firing said coating, applying to said face a coating of enamel in a color contrasting with that of the first coating, wiping the second coating from the bars only, and firing the plate to bake thereon the portion of said last mentioned coating borne by said characters.

3. The method of producing enameled metal signs, which consists in shaping a single sheet metal blank to form a unitary flat plate structure having portions cut therefrom to provide a pair of parallel hori-

zontally disposed bars and a plurality of sign characters of skeleton form located between and united at their tops and bottoms to said bars, and then successively applying to the plate a plurality of coatings of enamel, separately firing said coatings, the final coating being of a color presenting a contrast with that of the bars as previously coated and being removed from said bars before firing.

In testimony whereof, I affix my signature.

CHARLES KAPNER.